

## UNITED STATES PATENT OFFICE

2,640,000

## FLAMEPROOFING METHOD AND PRODUCT

Leslie P. Seyb, Painesville, and Clifford A. Neros,  
Willoughby, Ohio, assignors to Diamond Alkali  
Company, Cleveland, Ohio, a corporation of  
Delaware

No Drawing. Application June 7, 1947,  
Serial No. 753,358

8 Claims. (Cl. 117—76)

1

This invention relates to the impregnation of natural or synthetic cellulosic fibers and fabrics with flameproofing and water-repelling substances and to the flameproofed impregnated cellulosic materials obtained. More particularly, the invention relates to methods of applying impregnating substances to such fibers and fabrics, which methods result in treated materials of tensile strength and storage life comparable to untreated materials.

The invention, in general, contemplates the provision in stable relation upon a fibrous or fabric flammable material of flameproofing and water-repelling substances including both inorganic flame retardant substances, such as antimony oxide, and highly chlorinated organic substances, such as chlorinated paraffin, such substances being maintained in entirely stable relationship on the treated material at ordinary temperatures but being adapted to co-act in flame retarding relationship upon exposure of the treated materials to flame temperatures. In the following specification, the invention is described with relation to its application to woven fabric, such as cotton duck, it being understood, however, that any fibrous or woven material of cellulosic origin may be similarly treated and the advantages of the invention thus obtained.

The flameproofing of fabrics has heretofore been proposed; furthermore, the provision of fabric impregnated with an inorganic flame retardant substance, such as antimony oxide, combined with an organic flame retardant substance, such as highly chlorinated paraffin, is also known. These prior proposals have envisioned the inhibition of flaming at flame temperature both by the individual action of the flame retardant materials and by the combined chemical action of the two substances.

The prior art, however, has not provided an entirely satisfactory solution to the flameproofing of fabrics in that while the action of the materials applied to the fabrics has been satisfactory at flame temperatures, the flameproofing materials on the fabric have resulted in a tendering or weakening of treated fabrics at normal temperatures, especially after relatively extended periods of storage or use and particularly at mildly elevated temperatures or under conditions of exposure to sunlight, such as can be expected to be encountered in ordinary storage and use.

2

According to prior practice, inorganic materials, such as antimony oxide, and organic materials, such as chlorinated paraffin, are suspended or dispersed in a liquid medium either alone or with various added materials, such as resinous substances, designed to improve adherence of the flameproofing mixture to the fabric, dyes, fillers or the like, and such suspension is applied to the cloth. Thus, the mixture of inorganic materials, chlorinated material and solvent is in intimate contact with the interstices of the fibers and upon the solvent being removed, the two flame retardant materials remain in such relationship and in contact with each other on the finished fabric.

It is known that highly chlorinated organic materials, such as chlorinated paraffins, are somewhat unstable and tend, especially when heated, to dehydrochlorinate releasing hydrogen chloride; in fact, it is generally believed that at least part of the flameproofing character of the above-mentioned mixture lies in this property and in the subsequent reaction of antimony oxide with hydrogen chloride to form antimony oxychloride, which is characterized by notable inhibition of combustion. Accordingly, at flame temperatures the ready release of hydrogen chloride is desired, for whatever the theory of its action, it is known that flameproofing compositions which do not release hydrogen chloride at such temperatures are relatively inefficient.

The spontaneous release of hydrogen chloride from the chlorinated material on the fabric, which release takes place at an appreciable rate at ordinary temperatures of storage or use, is, however, quite another matter and results in a relatively substantial loss of tensile strength of prior art treated fabrics and in relatively short times. Various neutralizing substances, such as calcium carbonate, have been included in flameproofing materials for the purpose of nullifying the harmful effect of released hydrogen chloride but such modifications have also failed to produce a flameproofed fabric having satisfactory storage life.

As a result of the present invention, however, it is now appreciated that the intimate contact of the highly chlorinated organic substances with the fibers of the fabric is detrimental thereto, the hydrogen chloride released acting to tender or lessen the tensile strength of the cellulosic

materials. Decomposition of chlorinated materials results presumably in part from spontaneous action and in part from contact with the normal environment of such materials in storage or use, such as light, air and moisture. In addition, the inorganic flame retardant materials or impurities normally present therein, which heretofore have been in intimate contact with the highly chlorinated material, play a substantial role in this undesired production of hydrogen chloride.

The method of the present invention includes the application of the inorganic flame retardant substance and the chlorinated organic material to fabric in such a manner as normally to maintain said substances out of contact with each other and normally to maintain the chlorinated material out of contact with the fabric, while still permitting intimate contact to be readily established to produce flame inhibiting relationship at flame temperatures.

The present invention, which permits the maintenance of the fibers of the fabric out of contact with the chlorinated material during storage or use may be achieved by separating the fibers of the fabric from the chlorinated material with an auxiliary water-repellent, normally hydrogen chloride inert, film which, in addition to functioning as a screen between the chlorinated material and the fibers, binds the inorganic flame retardant substance within the interstices of the fibers. In addition to enhancing the storage life of the fabric, the auxiliary film, which is preferably water-repellent, improves the moisture-proof character of the treated fabric.

Application of the auxiliary film material may be achieved in a number of ways. If desired, the film forming material may be incorporated into a suspension of inorganic flame retardant material prior to application to the fabric in a manner to coat completely the particles of the inorganic material. This combination of inorganic material and film forming material may then be applied to the fabric to insure the complete coating of the fibers of the fabric. Then upon subsequent application of the chlorinated organic material to the thus initially treated fabric, the chlorinated material being preferably applied in a solvent therefor which is a non-solvent for the film material, a system will be obtained wherein the chlorinated material, though closely associated with the fabric and adapted to co-act with the inorganic flame retardant substance at flame temperatures, is nevertheless normally maintained out of actual contact with the fibers of the fabric and with the inorganic materials whereby decomposition of the chlorinated material and release of HCl at other than flame temperatures cannot deleteriously affect the fibers of the fabric.

It is also within the contemplation of the invention that suspended particles of inorganic flame retardant material may be coated with the film forming material, particles of chlorinated material may be similarly so coated and present in the same suspension, whereby a system is achieved wherein the inorganic and organic materials are maintained in separated relationship in suspension in the same solvent. The fabric is then contacted with a film forming material whereby the fibers of the fabric are essentially completely coated, whereupon the prepared suspension of coated inorganic and organic flame retardant material is applied to the thus treated fabric, achieving a finished material wherein as before, the flame retardant agents are separated

from each other and particularly the chlorinated organic material is separated from the fibers of the fabric. Upon reaching flame temperatures, however, the flame retardant materials co-act to inhibit flaming as described above.

Still another and the preferred method of achieving the desirable results of this invention contemplates the application to the fabric of the inorganic flame retardant material suspended in 10 a volatile solvent, followed by application of a film forming material thereto, and finally applying a solution of chlorinated material in a non-solvent for the film forming material. It will be seen that under the conditions of this aspect 15 of the invention, the desired normal separation of the flame retardant materials and the separation of chlorinated material from the fibers is again achieved, while also providing an environment for the flame retardant to co-act at flame 20 temperatures.

The inorganic flame retardant substance to be used in the practice of the present invention may comprise salts of antimony, arsenic, and bismuth, or salts of phosphoric, boric or stannic acids or mixtures thereof. In general, compounds of antimony, particularly antimony tri-oxide ( $Sb_2O_3$ ), are preferred. The highly chlorinated organic flame retardant substance may be any one of several types of chlorinated organic compounds, such as chlorinated oils of vegetable or animal origin, chlorinated paraffin wax, or wax-like substances. In general, it is preferred that the chlorinated substance be non-toxic to warm-blooded animals, readily soluble in organic solvents, and that such substance possess a low vapor pressure, while releasing substantial amounts of hydrogen chloride at flame temperatures. The preferred highly chlorinated organic substance for the practice of the present invention is a chlorinated paraffin wax containing between 40% and 70% of chemically combined chlorine, it also having been found advantageous to use mixtures of highly chlorinated paraffins, one component of such mixture containing about 40% of chemically combined chlorine and another component containing above 65% of chemically combined chlorine.

The film forming substance to be used in the practice of the present invention as a screen or barrier between the somewhat unstable chlorinated organic material and the fibers of the fabric, as well as the inorganic flameproofing material, may be drawn from a wide variety of film forming resinous materials which are characterized by substantial insolubility in at least one solvent in which the chlorinated material has substantial solubility. In addition, of course, in order to enhance the ultimate water-repellency of the fabric treated, the film forming screen material is preferably itself water-repellent when deposited as a film. Also, the film forming material must be readily decomposable at flame temperatures in order that the inorganic and organic flame retardant materials may co-act at such temperatures to inhibit burning of the fabric. At ordinary service temperatures, however, it is preferred that the film forming material be inert to conditions to which fabric may be exposed as well as to both the inorganic and organic constituents of the flameproofing composition.

In the following table are set forth various examples of resinous film forming substances which meet the above conditions; many other specific examples will occur to those skilled in

the art without departing from the scope of the invention herein.

oxide ( $Sb_2O_3$ ) 100 parts, urea-formaldehyde condensation product (50% solution) 72 parts, com-

Table "A"

| Film Forming Material  | Solvent            | Chlorinated Material | Solvent                          |
|------------------------|--------------------|----------------------|----------------------------------|
| Ethyl Cellulose        | Acetone            | Chlorinated Paraffin | Chain Hydrocarbons, <sup>1</sup> |
| Polyethylene           | Hot Xylol          | do                   | Cold Xylol.                      |
| Cellulose Acetate      | Acetone            | do                   | Chain Hydrocarbons, <sup>1</sup> |
| Styrene Resins         | Esters-Ketones     | do                   | Do, <sup>1</sup>                 |
| Polyvinyl Butyral      | Aliphatic Alcohols | do                   | Do, <sup>1</sup>                 |
| Methylmethacrylate     | Acetone            | do                   | Cyclohexane.                     |
| Ethylmethacrylate      | do                 | do                   | Do.                              |
| Iso-Propylmethacrylate | do                 | do                   | Hexene.                          |
| n-Butylmethacrylate    | do                 | do                   | Do.                              |
| n-Propylmethacrylate   | do                 | do                   | Do.                              |
| Iso-Butylmethacrylate  | do                 | do                   | Do.                              |

<sup>1</sup> Heptanes to light kerosene (duodecane) substantially no aromatics.

The film forming substance may be applied to the cloth in any of the previously described sequences of steps by any suitable means, such as hot rolling, calendering, flame spraying, solution spraying, brushing, doctoring, or the like.

It will be appreciated that the adoption of different chlorinated materials from chlorinated paraffin in the practice of the present invention may introduce slight variations in the information given in the table above. However, as stated hereinbefore, any film forming resin, especially the water insoluble members of such class of resins which is insoluble in a solvent in which the chlorinated material is soluble, may be employed herein. Also, it will be appreciated from the foregoing that, though there exist a number of variations which may be resorted to in the practice of the present method, it is in general preferred, to obtain the desired protection of the fibers of the fabric, that the film forming material be applied to the fabric prior to application thereto of the chlorinated material.

For a more complete understanding of the present invention and in order to enable those skilled in the art to practice the same, the following specific examples are offered, it being understood that the same are to be taken as illustrative only.

#### Example I

Bath I: Antimony oxide ( $Sb_2O_3$ ) 200 parts, urea-formaldehyde condensation product (50% solution) 72 parts, xylol 350 parts. Bath II: A 10% hot xylol solution of polyethylene having an average molecular weight of about 15,000. Bath III: Chlorinated paraffin wax containing 40% of chemically combined chlorine 120 parts, comminuted calcium carbonate 200 parts, urea-formaldehyde condensation product (50% solution) 26 parts, cold xylol 633 parts.

A heavy canvas material (14 ounce duck) is dipped in bath I and removed, dried at 190° F. for 30 minutes, and then dipped in bath II and dried at 190° F. for 30 minutes, and then dipped in bath III and dried at 190° F. for 30 minutes. The material is found to have increased in weight after the third dip by about 60% of the original weight of the untreated cloth. Using the standard fire test, E-11 of the Jeffersonville Quartermaster Depot, Specification No. 242, Section F-3, the following results are obtained as an average from several specimens tested: Duration of the flaming (seconds)—0; Length of char (inches)—2%.

#### Example II

(Olive drab colored coating) Bath I: Antimony

25 minuted calcium carbonate 100 parts, xylol 375 parts. Bath II: A 10% solution of polyethylene in hot xylol similar to that used in Example I. Bath III: Chromium oxide ( $Cr_2O_3$ ) 46 parts, yellow iron oxide 34 parts, red iron oxide 24 parts, Ramapo Blue (dye) 2½ parts, comminuted calcium carbonate 50 parts, copper naphthenate (8% solution in xylol) 45 parts, chlorinated paraffin wax containing 40% of chemically combined chlorine 100 parts, chlorinated paraffin wax containing 70% of chemically combined chlorine (70% solution on xylol) 60 parts, cold xylol 255 parts.

35 A heavy canvas material (14 ounce duck) is 30 dipped in bath I and dried at 190° F. for 30 minutes and is found to have increased in weight by 25.6% based on the original weight of the cloth. This is followed by dipping in bath II and drying at 190° F. for 30 minutes; after this drying, the 40 weight of the deposited film is 4.6% of the original weight of the untreated cloth. This is followed by dipping in bath III, drying at 190° F. for 30 minutes, following which the material has increased by 35.6% of the original weight of the untreated cloth, giving a total pickup from all three 45 baths of 65.8% based on the weight of the untreated cloth. A fire test made by the same specification as that used in Example I gives the following results: Duration of flaming (seconds) 50 1; length of char (inches) 3. An examination of the cross-section of this material shows that none of the materials contained in bath III penetrate the material which was applied in bath II and further that no pigmented portion is in contact 55 with the fibers of the canvas duck.

#### Example III

Using the same parts and proportions as in Example I for bath I, a 10% solution of methyl methacrylate in acetone for bath II, and the same proportions described in Example I for bath III, all dissolved (or in the case of calcium carbonate suspended) in cyclohexane, the procedure of Example I results in a water-repellent material having flame retardant properties similar to that of the product of Example I and having shelf and normal use life equal to untreated cloth.

70 While we have described in detail certain forms of our invention and certain specific examples of its practice, we do not wish to be understood as limiting ourselves to the use of such examples as we realize that changes within the scope of the invention are possible, and we further intend each step in the following claims to refer

to all equivalent steps for accomplishing the same result in substantially the same or equivalent manner, it being our purpose to cover our invention broadly in whatever form its principle may be utilized.

What is claimed is:

1. A fibrous cellulosic material of substantial flame-retardant properties comprising, in combination, a fibrous cellulosic base, a non-halogenated inorganic, flame-retardant substance deposited thereon, a resinous, organic, non-halogenated, heat-decomposable, film-forming substance overlaying said inorganic flame-retardant substance deposited upon said cellulosic base, and a highly chlorinated organic flame-retardant substance having a low vapor pressure, capable of releasing substantial amounts of hydrogen chloride at flame temperatures, deposited upon said film-forming substance so as to be maintained out of contact with said cellulosic base and said inorganic flame-retardant substance by means of said film-forming substance.

2. A fibrous cellulosic material having deposited thereon, a non-halogenated inorganic, flameproofing agent comprising antimony oxide ( $Sb_2O_3$ ), a heat-decomposable, non-halogenated, film-forming, resinous substance overlaying said inorganic flameproofing composition on said cellulosic material, and a highly chlorinated organic flame-retardant substance having a low vapor pressure, capable of releasing substantial amounts of hydrogen chloride at flame temperatures, deposited upon said film-forming substance, said chlorinated organic flame-retardant substance consisting essentially of chlorinated paraffin wax containing more than 40% of chemically combined chlorine.

3. A fibrous cellulosic material of substantial flame-retardant properties comprising, in combination, a fibrous cellulosic base, a non-halogenated inorganic, flame-retardant substance selected from the group consisting of antimony oxide, salts of antimony, arsenic, and bismuth, salts of phosphoric, boric, and stannic acids, and mixtures of said salts, deposited thereon, a film of a heat-decomposable, non-halogenated, film-forming, resinous solid selected from the group consisting of cellulose ethers, cellulose esters, polyethylene, polystyrene, polyvinyl butyral, and polyacrylic acid esters, overlaying said inorganic flame-retardant substance deposited upon said film, said highly chlorinated organic flame-retardant substance being selected from the group consisting of chlorinated vegetable oils, chlorinated animal oils, and chlorinated paraffin wax.

4. The article of claim 3 in which the inorganic flame-retardant substance is antimony oxide ( $Sb_2O_3$ ), the heat-decomposable, non-halogenated, film-forming, resinous solid is polyethylene, and the highly chlorinated organic flame-retardant substance is chlorinated paraffin wax containing from 40%-70% of chemically combined chlorine.

5. The method of flameproofing a fibrous cellulosic material, which includes the steps of (1) impregnating said material with a non-halogenated inorganic, flame-retardant substance, (2) depositing upon the thus-impregnated cellulosic material a film of a heat-decomposable, organic, non-halogenated, polymeric, film-forming, resinous substance inert to said inorganic flame-retardant substance and to highly chlorinated organic substances, thereby to form a screen between said inorganic flame-retardant substance and highly chlorinated organic substances sub-

sequently applied thereto, and (3) applying to the composite thus formed, a highly chlorinated organic flame-retardant substance having low vapor pressure, and capable of releasing substantial amounts of hydrogen chloride at flame temperatures.

6. The method of impregnating a fibrous cellulosic material with a flameproofing, water-repellent coating, which includes the steps of (1) impregnating said material with a substance selected from the group consisting of antimony trioxide, salts of antimony, arsenic, and bismuth, salts of phosphoric, boric, and stannic acids, and mixtures of said salts, (2) applying to the thus-impregnated material a solution of a heat-decomposable, organic, non-halogenated, film-forming, resinous solid selected from the group consisting of cellulose ethers, cellulose esters, polyethylene, polystyrene, polyvinyl butyral, and polyacrylic acid esters, (3) evaporating the solvent from the solution deposited upon said impregnated material to leave a film of said resinous solid overlaying said impregnated material, (4) applying to said film upon said impregnated material, a solution of a highly chlorinated organic flame-retardant substance selected from the group consisting of chlorinated vegetable oils, chlorinated animal oils, and chlorinated paraffin wax containing from 40%-70% of chemically combined chlorine, the solvent of said solution of said highly chlorinated organic substance being substantially a non-solvent for said film-forming, resinous solid, and (5) evaporating the solvent from said solution of said highly chlorinated organic substance applied to said film.

7. The method of impregnating a fibrous cellulosic material with a flame-retardant, water-repellent coating, which includes the steps of (1) impregnating said material with antimony trioxide, (2) applying to the thus-impregnated cellulosic material, a solution of a heat-decomposable, organic, non-halogenated, film-forming, resinous substance selected from the group consisting of cellulose ethers, cellulose esters, polyethylene, polystyrene, polyvinyl butyral, and polyacrylic acid esters, (3) evaporating the solvent from the solution applied to said impregnated material to deposit a film of said resinous substance upon said impregnated cellulosic material, (4) applying to said film a solution of chlorinated paraffin wax in a solvent which is substantially a non-solvent for said resinous, film-forming substance, said chlorinated paraffin wax containing from 40%-70% of chemically combined chlorine, and (5) evaporating the solvent from said solution of said chlorinated paraffin wax applied to said film.

8. The method of claim 7 in which said heat-decomposable, organic, non-halogenated, film-forming, resinous substance is polyethylene.

LESLIE P. SEYB.  
CLIFFORD A. NEROS.

65  
66  
67  
68  
69  
70  
71  
72  
73  
74  
75  
76  
77  
78  
79  
80  
81  
82  
83  
84  
85  
86  
87  
88  
89  
90  
91  
92  
93  
94  
95  
96  
97  
98  
99  
100  
101  
102  
103  
104  
105  
106  
107  
108  
109  
110  
111  
112  
113  
114  
115  
116  
117  
118  
119  
120  
121  
122  
123  
124  
125  
126  
127  
128  
129  
130  
131  
132  
133  
134  
135  
136  
137  
138  
139  
140  
141  
142  
143  
144  
145  
146  
147  
148  
149  
150  
151  
152  
153  
154  
155  
156  
157  
158  
159  
160  
161  
162  
163  
164  
165  
166  
167  
168  
169  
170  
171  
172  
173  
174  
175  
176  
177  
178  
179  
180  
181  
182  
183  
184  
185  
186  
187  
188  
189  
190  
191  
192  
193  
194  
195  
196  
197  
198  
199  
200  
201  
202  
203  
204  
205  
206  
207  
208  
209  
210  
211  
212  
213  
214  
215  
216  
217  
218  
219  
220  
221  
222  
223  
224  
225  
226  
227  
228  
229  
230  
231  
232  
233  
234  
235  
236  
237  
238  
239  
240  
241  
242  
243  
244  
245  
246  
247  
248  
249  
250  
251  
252  
253  
254  
255  
256  
257  
258  
259  
259  
260  
261  
262  
263  
264  
265  
266  
267  
268  
269  
270  
271  
272  
273  
274  
275  
276  
277  
278  
279  
280  
281  
282  
283  
284  
285  
286  
287  
288  
289  
290  
291  
292  
293  
294  
295  
296  
297  
298  
299  
300  
301  
302  
303  
304  
305  
306  
307  
308  
309  
310  
311  
312  
313  
314  
315  
316  
317  
318  
319  
320  
321  
322  
323  
324  
325  
326  
327  
328  
329  
330  
331  
332  
333  
334  
335  
336  
337  
338  
339  
340  
341  
342  
343  
344  
345  
346  
347  
348  
349  
350  
351  
352  
353  
354  
355  
356  
357  
358  
359  
360  
361  
362  
363  
364  
365  
366  
367  
368  
369  
370  
371  
372  
373  
374  
375  
376  
377  
378  
379  
380  
381  
382  
383  
384  
385  
386  
387  
388  
389  
390  
391  
392  
393  
394  
395  
396  
397  
398  
399  
400  
401  
402  
403  
404  
405  
406  
407  
408  
409  
410  
411  
412  
413  
414  
415  
416  
417  
418  
419  
420  
421  
422  
423  
424  
425  
426  
427  
428  
429  
430  
431  
432  
433  
434  
435  
436  
437  
438  
439  
440  
441  
442  
443  
444  
445  
446  
447  
448  
449  
450  
451  
452  
453  
454  
455  
456  
457  
458  
459  
460  
461  
462  
463  
464  
465  
466  
467  
468  
469  
470  
471  
472  
473  
474  
475  
476  
477  
478  
479  
480  
481  
482  
483  
484  
485  
486  
487  
488  
489  
490  
491  
492  
493  
494  
495  
496  
497  
498  
499  
500  
501  
502  
503  
504  
505  
506  
507  
508  
509  
510  
511  
512  
513  
514  
515  
516  
517  
518  
519  
520  
521  
522  
523  
524  
525  
526  
527  
528  
529  
530  
531  
532  
533  
534  
535  
536  
537  
538  
539  
540  
541  
542  
543  
544  
545  
546  
547  
548  
549  
550  
551  
552  
553  
554  
555  
556  
557  
558  
559  
559  
560  
561  
562  
563  
564  
565  
566  
567  
568  
569  
569  
570  
571  
572  
573  
574  
575  
576  
577  
578  
579  
579  
580  
581  
582  
583  
584  
585  
586  
587  
588  
589  
589  
590  
591  
592  
593  
594  
595  
596  
597  
598  
599  
600  
601  
602  
603  
604  
605  
606  
607  
608  
609  
609  
610  
611  
612  
613  
614  
615  
616  
617  
618  
619  
619  
620  
621  
622  
623  
624  
625  
626  
627  
628  
629  
629  
630  
631  
632  
633  
634  
635  
636  
637  
638  
639  
639  
640  
641  
642  
643  
644  
645  
646  
647  
648  
649  
649  
650  
651  
652  
653  
654  
655  
656  
657  
658  
659  
659  
660  
661  
662  
663  
664  
665  
666  
667  
668  
669  
669  
670  
671  
672  
673  
674  
675  
676  
677  
678  
679  
679  
680  
681  
682  
683  
684  
685  
686  
687  
688  
689  
689  
690  
691  
692  
693  
694  
695  
696  
697  
698  
699  
700  
701  
702  
703  
704  
705  
706  
707  
708  
709  
709  
710  
711  
712  
713  
714  
715  
716  
717  
718  
719  
719  
720  
721  
722  
723  
724  
725  
726  
727  
728  
729  
729  
730  
731  
732  
733  
734  
735  
736  
737  
738  
739  
739  
740  
741  
742  
743  
744  
745  
746  
747  
748  
749  
749  
750  
751  
752  
753  
754  
755  
756  
757  
758  
759  
759  
760  
761  
762  
763  
764  
765  
766  
767  
768  
769  
769  
770  
771  
772  
773  
774  
775  
776  
777  
778  
779  
779  
780  
781  
782  
783  
784  
785  
786  
787  
788  
789  
789  
790  
791  
792  
793  
794  
795  
796  
797  
798  
799  
800  
801  
802  
803  
804  
805  
806  
807  
808  
809  
809  
810  
811  
812  
813  
814  
815  
816  
817  
818  
819  
819  
820  
821  
822  
823  
824  
825  
826  
827  
828  
829  
829  
830  
831  
832  
833  
834  
835  
836  
837  
838  
839  
839  
840  
841  
842  
843  
844  
845  
846  
847  
848  
849  
849  
850  
851  
852  
853  
854  
855  
856  
857  
858  
859  
859  
860  
861  
862  
863  
864  
865  
866  
867  
868  
869  
869  
870  
871  
872  
873  
874  
875  
876  
877  
878  
879  
879  
880  
881  
882  
883  
884  
885  
886  
887  
888  
889  
889  
890  
891  
892  
893  
894  
895  
896  
897  
898  
899  
900  
901  
902  
903  
904  
905  
906  
907  
908  
909  
909  
910  
911  
912  
913  
914  
915  
916  
917  
918  
919  
919  
920  
921  
922  
923  
924  
925  
926  
927  
928  
929  
929  
930  
931  
932  
933  
934  
935  
936  
937  
938  
939  
939  
940  
941  
942  
943  
944  
945  
946  
947  
948  
949  
949  
950  
951  
952  
953  
954  
955  
956  
957  
958  
959  
959  
960  
961  
962  
963  
964  
965  
966  
967  
968  
969  
969  
970  
971  
972  
973  
974  
975  
976  
977  
978  
979  
979  
980  
981  
982  
983  
984  
985  
986  
987  
988  
989  
989  
990  
991  
992  
993  
994  
995  
996  
997  
998  
999  
1000  
1001  
1002  
1003  
1004  
1005  
1006  
1007  
1008  
1009  
1009  
1010  
1011  
1012  
1013  
1014  
1015  
1016  
1017  
1018  
1019  
1019  
1020  
1021  
1022  
1023  
1024  
1025  
1026  
1027  
1028  
1029  
1029  
1030  
1031  
1032  
1033  
1034  
1035  
1036  
1037  
1038  
1039  
1039  
1040  
1041  
1042  
1043  
1044  
1045  
1046  
1047  
1048  
1049  
1049  
1050  
1051  
1052  
1053  
1054  
1055  
1056  
1057  
1058  
1059  
1059  
1060  
1061  
1062  
1063  
1064  
1065  
1066  
1067  
1068  
1069  
1069  
1070  
1071  
1072  
1073  
1074  
1075  
1076  
1077  
1078  
1079  
1079  
1080  
1081  
1082  
1083  
1084  
1085  
1086  
1087  
1088  
1089  
1089  
1090  
1091  
1092  
1093  
1094  
1095  
1096  
1097  
1098  
1099  
1100  
1101  
1102  
1103  
1104  
1105  
1106  
1107  
1108  
1109  
1109  
1110  
1111  
1112  
1113  
1114  
1115  
1116  
1117  
1118  
1119  
1119  
1120  
1121  
1122  
1123  
1124  
1125  
1126  
1127  
1128  
1129  
1129  
1130  
1131  
1132  
1133  
1134  
1135  
1136  
1137  
1138  
1139  
1139  
1140  
1141  
1142  
1143  
1144  
1145  
1146  
1147  
1148  
1149  
1149  
1150  
1151  
1152  
1153  
1154  
1155  
1156  
1157  
1158  
1159  
1159  
1160  
1161  
1162  
1163  
1164  
1165  
1166  
1167  
1168  
1169  
1169  
1170  
1171  
1172  
1173  
1174  
1175  
1176  
1177  
1178  
1179  
1179  
1180  
1181  
1182  
1183  
1184  
1185  
1186  
1187  
1188  
1189  
1189  
1190  
1191  
1192  
1193  
1194  
1195  
1196  
1197  
1198  
1199  
1200  
1201  
1202  
1203  
1204  
1205  
1206  
1207  
1208  
1209  
1209  
1210  
1211  
1212  
1213  
1214  
1215  
1216  
1217  
1218  
1219  
1219  
1220  
1221  
1222  
1223  
1224  
1225  
1226  
1227  
1228  
1229  
1229  
1230  
1231  
1232  
1233  
1234  
1235  
1236  
1237  
1238  
1239  
1239  
1240  
1241  
1242  
1243  
1244  
1245  
1246  
1247  
1248  
1249  
1249  
1250  
1251  
1252  
1253  
1254  
1255  
1256  
1257  
1258  
1259  
1259  
1260  
1261  
1262  
1263  
1264  
1265  
1266  
1267  
1268  
1269  
1269  
1270  
1271  
1272  
1273  
1274  
1275  
1276  
1277  
1278  
1279  
1279  
1280  
1281  
1282  
1283  
1284  
1285  
1286  
1287  
1288  
1289  
1289  
1290  
1291  
1292  
1293  
1294  
1295  
1296  
1297  
1298  
1299  
1300  
1301  
1302  
1303  
1304  
1305  
1306  
1307  
1308  
1309  
1309  
1310  
1311  
1312  
1313  
1314  
1315  
1316  
1317  
1318  
1319  
1319  
1320  
1321  
1322  
1323  
1324  
1325  
1326  
1327  
1328  
1329  
1329  
1330  
1331  
1332  
1333  
1334  
1335  
1336  
1337  
1338  
1339  
1339  
1340  
1341  
1342  
1343  
1344  
1345  
1346  
1347  
1348  
1349  
1349  
1350  
1351  
1352  
1353  
1354  
1355  
1356  
1357  
1358  
1359  
1359  
1360  
1361  
1362  
1363  
1364  
1365  
1366  
1367  
1368  
1369  
1369  
1370  
1371  
1372  
1373  
1374  
1375  
1376  
1377  
1378  
1379  
1379  
1380  
1381  
1382  
1383  
1384  
1385  
1386  
1387  
1388  
1389  
1389  
1390  
1391  
1392  
1393  
1394  
1395  
1396  
1397  
1398  
1399  
1400  
1401  
1402  
1403  
1404  
1405  
1406  
1407  
1408  
1409  
1409  
1410  
1411  
1412  
1413  
1414  
1415  
1416  
1417  
1418  
1419  
1419  
1420  
1421  
1422  
1423  
1424  
1425  
1426  
1427  
1428  
1429  
1429  
1430  
1431  
1432  
1433  
1434  
1435  
1436  
1437  
1438  
1439  
1439  
1440  
1441  
1442  
1443  
1444  
1445  
1446  
1447  
1448  
1449  
1449  
1450  
1451  
1452  
1453  
1454  
1455  
1456  
1457  
1458  
1459  
1459  
1460  
1461  
1462  
1463  
1464  
1465  
1466  
1467  
1468  
1469  
1469  
1470  
1471  
1472  
1473  
1474  
1475  
1476  
1477  
1478  
1479  
1479  
1480  
1481  
1482  
1483  
1484  
1485  
1486  
1487  
1488  
1489  
1489  
1490  
1491  
1492  
1493  
1494  
1495  
1496  
1497  
1498  
1499  
1500  
1501  
1502  
1503  
1504  
1505  
1506  
1507  
1508  
1509  
1509  
1510  
1511  
1512  
1513  
1514  
1515  
1516  
1517  
1518  
1519  
1519  
1520  
1521  
1522  
1523  
1524  
1525  
1526  
1527  
1528  
1529  
1529  
1530  
1531  
1532  
1533  
1534  
1535  
1536  
1537  
1538  
1539  
1539  
1540  
1541  
1542  
1543  
1544  
1545  
1546  
1547  
1548  
1549  
1549  
1550  
1551  
1552  
1553  
1554  
1555  
1556  
1557  
1558  
1559  
1559  
1560  
1561  
1562  
1563  
1564  
1565  
1566  
1567  
1568  
1569  
1569  
1570  
1571  
1572  
1573  
1574  
1575  
1576  
1577  
1578  
1579  
1579  
1580  
1581  
1582  
1583  
1584  
1585  
1586  
1587  
1588  
1589  
1589  
1590  
1591  
1592  
1593  
1594  
1595  
1596  
1597  
1598  
1599  
1600  
1601  
1602  
1603  
1604  
1605  
1606  
1607  
1608  
1609  
1609  
1610  
1611  
1612  
1613  
1614  
1615  
1616  
1617  
1618  
1619  
1619  
1620  
1621  
1622  
1623  
1624  
1625  
1626  
1627  
1628  
1629  
1629  
1630  
1631  
1632  
1633  
1634  
1635  
1636  
1637  
1638  
1639  
1639  
1640  
1641  
1642  
1643  
1644  
1645  
1646  
1647  
1648  
1649  
1649  
1650  
1651  
1652  
1653  
1654  
1655  
1656  
1657  
1658  
1659  
1659  
1660  
1661  
1662  
1663  
1664  
1665  
1666  
1667  
1668  
1669  
1669  
1670  
1671  
1672  
1673  
1674  
1675  
1676  
1677  
1678  
1679  
1679  
1680  
1681  
1682  
1683  
1684  
1685  
1686  
1687  
1688  
1689  
1689  
1690  
1691  
1692  
1693  
1694  
1695  
1696  
1697  
1698  
1699  
1700  
1701  
1702  
1703  
1704<br

2,640,000

9

UNITED STATES PATENTS

| Number    | Name            | Date           |
|-----------|-----------------|----------------|
| 2,380,775 | Meyer           | July 31, 1945  |
| 2,416,447 | Laughlin et al. | Feb. 25, 1947  |
| 2,424,386 | Czezowitzka     | July 22, 1947  |
| 2,427,997 | White           | Sept. 23, 1947 |
| 2,428,716 | McGill et al.   | Oct. 7, 1947   |
| 2,431,001 | Sullivan        | Nov. 18, 1947  |
| 2,494,391 | Johnson et al.  | Jan. 10, 1950  |

10

FOREIGN PATENTS

| Number  | Country       | Date          |
|---------|---------------|---------------|
| 552,909 | Great Britain | Apr. 29, 1943 |

5 OTHER REFERENCES

Little, "Flameproofing Textile Fabrics," A. C. S., Monograph Series No. 104, published 1947, pages 240, 241, 249.